

Sept. 15, 1942.

D. G. MAGILL

2,296,171

METHOD OF PRODUCING SHEET MATERIAL

Filed Nov. 13, 1939



INVENTOR  
Donald G. Magill  
BY  
Drew D. Hollingshead  
Charles H. Cripe  
ATTORNEYS

## UNITED STATES PATENT OFFICE

2,296,171

## METHOD OF PRODUCING SHEET MATERIAL

Donald G. Magill, Great Neck, N. Y., assignor to  
American Can Company, New York, N. Y., a  
corporation of New Jersey

Application November 13, 1939, Serial No. 304,275

2 Claims. (Cl. 154—40)

The present invention relates to a method of producing sheet or web base material from which fibre containers and the like may be made and has particular reference to such a material of a laminated and moistureproof nature.

An object of the invention is the provision of a method of producing a moistureproof laminated sheet or web material wherein a film of micro-crystalline or amorphous wax is applied to a preferably thin cellulosic impervious or impermeable web such as "Cellophane" or glassine or to a non-cellulosic impervious web such as "Pliofilm" or "Koro seal" and this web applied under pressure and at room temperature to a heavier pervious or permeable fibrous base sheet or strip such as chipboard, kraft paper, or the like, thereby bonding them together in a manner which extrudes the wax coating on the impervious web into the top fibre of the pervious base without penetrating through the wax film, thus effecting a firm adherence and film continuity between the layers to produce a laminated moistureproof web from which containers or the like may be made.

Another object is the provision of such a method of producing a laminated moistureproof material wherein the micro-crystalline wax is applied to the impervious web in a molten state and is cooled to a degree well below its point of solidification prior to the impervious web being united with the pervious base strip so that penetration of the wax film by the fibres of the base stock will be prevented when the layers are pressed together.

Another object is the provision of a method of this character wherein the micro-crystalline wax applied to the impervious web is metered in order to produce an accurately reduced minimum film capable of maximum moisture resistance.

Numerous other objects and advantages of the invention will be apparent as it is better understood from the following description, which, taken in connection with the accompanying drawing, discloses a preferred embodiment thereof.

Referring to the drawing:

Figure 1 is a longitudinal vertical sectional view illustrating an apparatus for carrying out the various steps of the instant method invention, the view also showing web layers of material in place in the apparatus; and

Fig. 2 is an enlarged detail of a metering rod used in the apparatus.

In a preferred embodiment of the invention a preferably thin web A of impervious material, such as glassine, "Cellophane," or other treated materials, is coated on one surface with a metered

uniform film of micro-crystalline or amorphous wax in a molten state maintained at approximately 180° F. Immediately after its application to the web the wax coating is cooled to a degree well below its point of solidification, such as for example, to approximately 70° F.

The wax coated impervious web A is then brought into contact with a preferably heavier pervious fibre base strip B such as chipboard, kraft paper or the like, with the wax film interposed therebetween. While these layers are so aligned they are subjected at room temperature (approximately 70° F.) to a relatively high pressure of approximately 3500 pounds. As shown in the drawing this pressure is exerted at the nip of the rolls. This pressure unites the impervious web A with the pervious strip or web B in a permanent bond and in a manner which extrudes the wax film of the impervious web into the interstices surrounding the top fibres of the pervious web without the top fibres penetrating through the wax film. This preserves the continuity of the film and thereby insures higher moisture resistance, since the film remains unbroken, and at the same time results in a firm adherence between the webs. Such a laminated moistureproof material has been found to be ideal for the manufacture of fibre containers for holding deliquescent granulated or powdered products which may be packed and safeguarded against moisture infecting conditions.

One form of apparatus as disclosed in the drawing for carrying out the steps of this method invention includes a main frame 11 which at one end is formed with brackets 12 carrying a cross rod 13 on which a roll 14 of the impervious web A is mounted. The web A extends over a guide bar 16 carried in side brackets 17 formed on the frame 11 and then passes through a coating device 18 which is disposed adjacent the guide bar.

The coating device includes a pair of upper and lower rollers 21, 22 between which the web passes and which serve as feed rollers for unreeling the web from its roll 14 and for advancing it along its path of travel. These rollers are continuously rotated in any suitable manner.

The lower feed roller 22 is also used as an applying roller and rotates in a molten bath of micro-crystalline or amorphous wax 23 retained in a reservoir 24 formed as an integral part of the main frame 11. Thus as the roller revolves, it carries the molten wax up out of the reservoir and applies it to the advancing web. The quantity of wax thus applied is preferably in excess

of that actually needed so that this excess may be reduced to a uniform film of predetermined thickness by a metering rod which will be hereinafter explained.

The wax before application to the web is maintained in a molten state by suitable heating elements disposed under the reservoir. These heating elements are preferably gas burners 26 which are connected into a main supply pipe 27 which leads to a suitable source of gas supply.

The upper feed roller 21 is also used as a pressure roller which presses the web against the applying roller 22. This pressure roller is maintained in a heated condition to prevent chilling of the newly applied hot wax. This heating effect is brought about by the circulation of steam through the roller and suitable circulation pipes 28 connecting with the interior of the roller are provided for this purpose.

The metering rod hereinbefore mentioned and broadly indicated by the numeral 31, is disposed adjacent the web exit side of the coating device just explained. This rod includes a preferably round stationary crossbar 32 (Fig. 2) the ends of which are carried in brackets 33 bolted to the side walls of the wax reservoir 24. The brackets are formed to hold the bar over the reservoir. Around the crossbar there is wrapped in helical fashion a round wire 34 of predetermined gauge which depends upon the degree of metering necessary, i. e., the thickness of the film desired. This wire when viewed in cross section as in Fig. 2 sets off a plurality of ridges 35 having spaces 36 therebetween.

Thus the freshly wax-coated web A as it leaves the coating device, glides over the metering bar 31 in contact with the helically wound wire 34. The wire thus scrapes off all wax except that which passes through the openings 36 between the ridges 35 of the wire and thereby leaves a plurality of small parallel and spaced wax ridges on the web surface. The excess wax falls back into the reservoir. Since the wax is still in a fluid state when this metering is done it immediately flows or spreads laterally into a film of uniform thickness instead of remaining in the series of parallel ridges as might be expected. This scraping action of the metering rod accurately reduces the wax on the web to a minimum film which is capable of maximum moisture resistance, this being a predetermined factor and obtained in practice by the gauge of the metering wire used in order to provide the proper size of openings 36.

Cooling of the wax film on the web A is preferably effected by air jets, indicated by the numeral 41 and which are projected against the wax covered surface of the web as the latter advances along its path of travel. These air jets issue from a spray head 42 carried on the upper end of an air pipe 43 which extends up through an aperture 44 formed in the main frame 11. The air pipe leads to any suitable source of supply of compressed air. A valve 45 in the air pipe is provided to manually control the volume of the air passing through the jets 41.

After the cooling operation of the wax coated web A, this web moves forward to meet the base strip B which is now introduced into the path of travel of the coated web. The base strip B is preferably unreeled from a roll 47 which is supported on a cross-rod 48 carried in the main frame 11. The base strip passes up and over the lower roller of a pair of pressure rollers 51, 52 and thus comes into contact with the

advancing wax coated web A and both web layers, in superimposed position, thereupon pass between the rollers.

The rollers 51, 52 are mounted on cross-shafts 53, 54 carried in brackets 55 formed on the main frame 11. These rollers are continuously rotated in any suitable manner. It is these pressure rollers that exert the high pressure at room temperature on the webs passing between and thus unite the web layers in a permanent bond. The pressure on these rollers may be exerted in any suitable manner.

The single web of moistureproof laminated and bonded material thus produced and indicated by the numeral 57 is advanced toward the discharge end of the apparatus and is wound on a reel or discharged to any suitable place of deposit. This discharge of the web as it is produced is effected by a pair of feed rollers 61, 62 between which the web passes. The rollers are mounted on continuously rotating cross-shafts 63, 64 which are carried in side frames 65 formed on the main frame 11.

While the drawing and the foregoing description disclose the production of a two ply web material by joining the impervious web A and the pervious fibre base strip B, it should be understood that more than a single web A or a single strip B could be used and a multiple layer or ply web material could be obtained if more laminations are desired. Furthermore, either the number of layers of either the web A or B may be increased without maintaining the same relationship of a single layer A for a single strip B. This will depend somewhat upon the purpose for which the multiple layer stock will be subsequently utilized.

It is thought that the invention and many of its attendant advantages will be understood from the foregoing description, and it will be apparent that various changes may be made in the steps of the process described and their order of accomplishment without departing from the spirit and scope of the invention or sacrificing all of its material advantages, the process hereinbefore described being merely a preferred embodiment thereof.

I claim:

1. A method of producing laminated sheets for the manufacture of moistureproof fibre containers having an inner impervious layer sheet, which method comprises coating a thin impervious carrier sheet selected from a class consisting of rubber hydrochloride, regenerated and hydrated cellulose, and vinyl resin, with an adhesive film of molten micro-crystalline wax, cooling said applied film of wax to a degree well below its point of solidification to solidify the same, bringing said wax coated impervious sheet into contact with a heavier permeable fibrous base sheet with the wax coating interposed therebetween, and then uniting said sheets by subjecting them to high pressure to permanently bond said sheets together by means of said adhesive wax film to produce a laminated moisture-proof sheet material for the manufacture of said fibre containers, said pressure being sufficiently high to extrude the solidified wax coating on the impervious sheet into the top fibres of the permeable base sheet, the cooling and solidification of the wax preventing the top fibres of said base sheet from penetrating through the wax film, thereby effecting an adherence and continuity of wax film between said sheets to produce a composite laminated moistureproof sheet.

2. A method of producing laminated sheets for the manufacture of moistureproof fibre containers having an inner impervious layer sheet, which method comprises coating a thin impervious carrier sheet selected from a class consisting of rubber hydrochloride, regenerated and hydrated cellulose, and vinyl resin, with an adhesive film of molten micro-crystalline wax, metering said wax coating into a film of predetermined uniform thickness, cooling said applied film of wax to a degree well below its point of solidification to solidify the same, bringing said wax coated impervious sheet into contact with a heavier permeable fibrous base sheet with the wax coating interposed therebetween, and 15

then uniting said sheets by subjecting them to high pressure to permanently bond said sheets together by means of said adhesive wax film to produce a laminated moistureproof sheet material for the manufacture of said fibre containers, said pressure being sufficiently high to extrude the solidified wax coating on the impervious sheet into the top fibres of the permeable base sheet, the cooling and solidification of the wax preventing the top fibres of said base sheet from penetrating through the wax film, thereby effecting an adherence and continuity of wax film between said sheets to produce a composite laminated moistureproof sheet.

DONALD G. MAGILL.